



US008851208B2

(12) **United States Patent**  
**Scott**

(10) **Patent No.:** **US 8,851,208 B2**  
(45) **Date of Patent:** **Oct. 7, 2014**

(54) **CUTTING ELEMENTS INCLUDING ADHESION MATERIALS, EARTH-BORING TOOLS INCLUDING SUCH CUTTING ELEMENTS, AND RELATED METHODS**

(71) Applicant: **Baker Hughes Incorporated**, Houston, TX (US)

(72) Inventor: **Danny E. Scott**, Montgomery, TX (US)

(73) Assignee: **Baker Hughes Incorporated**, Houston, TX (US)

(\*) Notice: Subject to any disclaimer, the term of this patent is extended or adjusted under 35 U.S.C. 154(b) by 0 days.

(21) Appl. No.: **14/062,133**

(22) Filed: **Oct. 24, 2013**

(65) **Prior Publication Data**

US 2014/0048341 A1 Feb. 20, 2014

**Related U.S. Application Data**

(63) Continuation of application No. 12/751,520, filed on Mar. 31, 2010, now Pat. No. 8,573,333.

(60) Provisional application No. 61/165,382, filed on Mar. 31, 2009.

(51) **Int. Cl.**

**E21B 10/46** (2006.01)

**E21B 10/573** (2006.01)

**E21B 10/55** (2006.01)

**B22F 5/00** (2006.01)

(52) **U.S. Cl.**

CPC ..... **E21B 10/5735** (2013.01); **B22F 2998/00** (2013.01); **E21B 10/55** (2013.01); **B22F 2005/001** (2013.01)

USPC ..... **175/434**; 175/432

(58) **Field of Classification Search**

CPC ... E21B 10/567; E21B 10/5735; E21B 10/46; E21B 10/55; C21C 1/1068; C22C 26/00; C22C 2204/00

USPC ..... 175/432, 434  
See application file for complete search history.

(56)

**References Cited**

U.S. PATENT DOCUMENTS

3,745,623 A 7/1973 Rocco et al.  
4,151,686 A 5/1979 Lee et al.

(Continued)

FOREIGN PATENT DOCUMENTS

JP 59219500 A 12/1984  
WO 9323204 A1 11/1993

(Continued)

OTHER PUBLICATIONS

International Search Report for International Application No. PCT/US2010/029320 mailed Jun. 29, 2010, 3 pages.

(Continued)

*Primary Examiner* — Jennifer H Gay

(74) *Attorney, Agent, or Firm* — TraskBritt

(57)

**ABSTRACT**

A cutting element for an earth-boring drill bit may include a thermally stable cutting table comprising a polycrystalline diamond material. The polycrystalline diamond material may consist essentially of a matrix of diamond particles bonded to one another and a silicon, silicon carbide, or silicon and silicon carbide material located within interstitial spaces among interbonded diamond particles of the matrix of diamond particles. The cutting table may be at least substantially free of Group VIII metal or alloy catalyst material. The cutting element may further include a substrate and an adhesion material between and bonded to the cutting table and the substrate. The adhesion material may include diamond particles bonded to one another and to the cutting table and the substrate after formation of the preformed cutting table.

**20 Claims, 3 Drawing Sheets**



|                              |                         |                       |                                                                                                                                    |               |                   |                   |                  |  |
|------------------------------|-------------------------|-----------------------|------------------------------------------------------------------------------------------------------------------------------------|---------------|-------------------|-------------------|------------------|--|
| (56)                         | <b>References Cited</b> |                       |                                                                                                                                    |               |                   |                   |                  |  |
| <b>U.S. PATENT DOCUMENTS</b> |                         |                       |                                                                                                                                    |               |                   |                   |                  |  |
| 4,224,380 A                  | 9/1980                  | Bovenkerk et al.      | 8,573,333 B2 *                                                                                                                     | 11/2013       | Scott .....       | 175/434           |                  |  |
| RE32,380 E                   | 3/1987                  | Wentorf               | 2001/0037609 A1                                                                                                                    | 11/2001       | Jensen et al.     |                   |                  |  |
| 4,766,040 A                  | 8/1988                  | Hillert et al.        | 2003/0129780 A1                                                                                                                    | 7/2003        | Auberton-Herve    |                   |                  |  |
| 4,793,828 A                  | 12/1988                 | Burnand               | 2003/0183426 A1                                                                                                                    | 10/2003       | Griffin et al.    |                   |                  |  |
| 5,020,394 A                  | 6/1991                  | Nakamura et al.       | 2003/0196385 A1                                                                                                                    | 10/2003       | Middlemiss        |                   |                  |  |
| 5,127,923 A                  | 7/1992                  | Bunting et al.        | 2004/0172885 A1                                                                                                                    | 9/2004        | Middlemiss        |                   |                  |  |
| 5,435,403 A *                | 7/1995                  | Tibbitts .....        | 175/432                                                                                                                            |               | 2005/0115744 A1   | 6/2005            | Griffin et al.   |  |
| 5,469,927 A                  | 11/1995                 | Griffin               |                                                                                                                                    |               | 2006/0060390 A1   | 3/2006            | Eyre             |  |
| 5,486,137 A                  | 1/1996                  | Flood et al.          |                                                                                                                                    |               | 2006/0060391 A1   | 3/2006            | Eyre et al.      |  |
| 5,743,346 A                  | 4/1998                  | Flood et al.          |                                                                                                                                    |               | 2006/0086540 A1   | 4/2006            | Griffin et al.   |  |
| 5,950,747 A *                | 9/1999                  | Tibbitts et al. ..... | 175/432                                                                                                                            |               | 2007/0023206 A1   | 2/2007            | Keshavan         |  |
| 6,021,859 A *                | 2/2000                  | Tibbitts et al. ..... | 175/431                                                                                                                            |               | 2007/0181348 A1   | 8/2007            | Lancaster et al. |  |
| 6,065,552 A                  | 5/2000                  | Scott et al.          |                                                                                                                                    |               | 2008/0085407 A1   | 4/2008            | Cooley et al.    |  |
| 6,189,634 B1                 | 2/2001                  | Bertagnolli et al.    |                                                                                                                                    |               | 2008/0115421 A1 * | 5/2008            | Sani .....       |  |
| 6,258,139 B1                 | 7/2001                  | Jensen                |                                                                                                                                    |               | 2008/0206576 A1   | 8/2008            | Qian et al.      |  |
| 6,447,560 B2                 | 9/2002                  | Jensen et al.         |                                                                                                                                    |               | 2008/0230280 A1   | 9/2008            | Keshavan et al.  |  |
| 6,544,308 B2                 | 4/2003                  | Griffin et al.        |                                                                                                                                    |               | 2009/0152018 A1   | 6/2009            | Sani             |  |
| 6,601,662 B2                 | 8/2003                  | Matthias et al.       |                                                                                                                                    |               | 2009/0313908 A1   | 12/2009           | Zhang et al.     |  |
| 6,846,341 B2                 | 1/2005                  | Middlemiss            |                                                                                                                                    |               | 2010/0012389 A1   | 1/2010            | Zhang et al.     |  |
| 6,986,297 B2                 | 1/2006                  | Scott                 |                                                                                                                                    |               | 2010/0126779 A1   | 5/2010            | Corbett et al.   |  |
| 7,350,601 B2                 | 4/2008                  | Belnap et al.         |                                                                                                                                    |               | 2010/0146865 A1   | 6/2010            | Sato et al.      |  |
| 7,377,341 B2                 | 5/2008                  | Middlemiss et al.     |                                                                                                                                    |               | 2010/0243337 A1   | 9/2010            | Scott            |  |
| 7,407,012 B2                 | 8/2008                  | Keshavan et al.       |                                                                                                                                    |               | 2010/0300767 A1   | 12/2010           | Cariveau et al.  |  |
| 7,462,003 B2                 | 12/2008                 | Middlemiss            |                                                                                                                                    |               | 2011/0042147 A1   | 2/2011            | Fang et al.      |  |
| 7,473,287 B2                 | 1/2009                  | Belnap et al.         |                                                                                                                                    |               | 2011/0259648 A1 * | 10/2011           | Sani .....       |  |
| 7,475,744 B2                 | 1/2009                  | Pope                  |                                                                                                                                    |               | 2012/0000136 A1 * | 1/2012            | Sani .....       |  |
| 7,506,698 B2                 | 3/2009                  | Eyre et al.           | WO                                                                                                                                 | 2004106003 A1 | 12/2004           | 175/428           |                  |  |
| 7,517,589 B2                 | 4/2009                  | Eyre                  | WO                                                                                                                                 | 2004106004 A1 | 12/2004           | 51/295            |                  |  |
| 7,533,740 B2                 | 5/2009                  | Zhang et al.          | WO                                                                                                                                 | 2005110648 A2 | 11/2005           | 2013/0313027 A1 * |                  |  |
| 7,608,333 B2                 | 10/2009                 | Eyre                  | FOREIGN PATENT DOCUMENTS                                                                                                           |               |                   |                   |                  |  |
| 7,628,234 B2                 | 12/2009                 | Middlemiss            | OTHER PUBLICATIONS                                                                                                                 |               |                   |                   |                  |  |
| 7,681,669 B2                 | 3/2010                  | Cannon et al.         | International Written Opinion for International Application No. PCT/US2010/029320 issued Jun. 29, 2011, 6 pages.                   |               |                   |                   |                  |  |
| 7,726,421 B2                 | 6/2010                  | Middlemiss            | International Preliminary Report on Patentability for International Application No. PCT/US2010/029320 dated Oct. 4, 2011, 6 pages. |               |                   |                   |                  |  |
| 7,754,333 B2                 | 7/2010                  | Eyre et al.           | * cited by examiner                                                                                                                |               |                   |                   |                  |  |
| 7,942,219 B2                 | 5/2011                  | Keshavan et al.       |                                                                                                                                    |               |                   |                   |                  |  |
| 7,998,573 B2                 | 8/2011                  | Qian et al.           |                                                                                                                                    |               |                   |                   |                  |  |
| 8,034,136 B2 *               | 10/2011                 | Sani .....            | 51/293                                                                                                                             |               |                   |                   |                  |  |

**FIG. 1A****FIG. 1****FIG. 1B**



FIG. 2



FIG. 3



FIG. 4A

FIG. 4



FIG. 5



FIG. 6

## 1

**CUTTING ELEMENTS INCLUDING  
ADHESION MATERIALS, EARTH-BORING  
TOOLS INCLUDING SUCH CUTTING  
ELEMENTS, AND RELATED METHODS**

**CROSS-REFERENCE TO RELATED  
APPLICATIONS**

This application is a continuation of U.S. patent application Ser. No. 12/751,520, filed Mar. 31, 2010, now U.S. Pat. No. 8,573,333, issued on Nov. 5, 2013, which is a utility conversion of U.S. Provisional Patent Application Ser. No. 61/165,382, filed Mar. 31, 2009, for "Methods For Bonding Preformed Cutting Tables to Cutting Element Substrates and Cutting Elements Formed by Such Processes," the disclosure of each of which is incorporated in this application in its entirety by this reference.

**FIELD**

The present disclosure relates generally to cutting elements, or cutters, for use with earth-boring drill bits and, more specifically, to cutting elements that include thermally stable, preformed superabrasive cutting tables adhered to substrates with diamond. The present disclosure also relates to methods for manufacturing such cutting elements, as well as to earth-boring drill bits that include such cutting elements.

**BACKGROUND**

Conventional polycrystalline diamond compact (PDC) cutting elements include a cutting table and a substrate. The substrate conventionally comprises a metal material, such as tungsten carbide, to enable robust coupling of the PDC cutting elements to a bit body. The cutting table typically includes randomly oriented, mutually bonded diamond (or, sometimes, cubic boron nitride (CBN)) particles that have also been adhered to the substrate on which the cutting table is formed, under extremely high-temperature, high-pressure (HTHP) conditions. Cobalt binders, also known as catalysts, have been widely used to initiate bonding of superabrasive particles to one another and to the substrates. Although the use of cobalt in PDC cutting elements has been widespread, PDC cutting elements having cutting tables that include cobalt binders are not thermally stable at the typically high operating temperatures to which the cutting elements are subjected due to the greater coefficient of thermal expansion of the cobalt relative to the superabrasive particles and, further, because the presence of cobalt tends to initiate back-graphitization of the diamond in the cutting table when a temperature above about 750° C. is reached. As a result, the presence of the cobalt results in premature wearing of and damage to the cutting table.

A number of different approaches have been taken to enhance the thermal stability of polycrystalline diamond and CBN cutting tables. One type of thermally stable cutting table that has been developed includes polycrystalline diamond sintered with a carbonate binder, such as a Mg, Ca, Sr, or Ba carbonate binder. The use of a carbonate binder increases the pressure and/or temperature required to actually bind diamond particles to one another, however. Consequently, the diameters of PDC cutting elements that include carbonate binders lack an integral carbide support or substrate and are typically much smaller than the diameters of PDC cutting elements that are manufactured with cobalt.

Another type of thermally stable cutting table is a PDC from which the cobalt binder has been removed, such as by

## 2

acid leaching or electrolytic removal. Such cutting elements have a tendency to be somewhat fragile, however, due to their lack of an integral carbide support or substrate and, in part, due to the removal of substantially all of the cobalt binder, which may result in a cutting table with a relatively low diamond density. Consequently, the practical size of a cutting table from which the cobalt may be effectively removed is limited.

Yet another type of thermally stable cutting table is similar to that described in the preceding paragraph, but the pores resulting from removal of the cobalt have been filled with silicon and/or silicon carbide. Examples of this type of cutting element are described in U.S. Pat. Nos. 4,151,686 and 4,793,828. Such cutting tables are more robust than those from which the cobalt has merely leached, but the silicon precludes easy attachment of the cutting table to a supporting substrate.

**SUMMARY**

20 The present disclosure includes embodiments of methods for adhering thermally stable diamond cutting tables to cutting element substrates. As used herein, the phrase "thermally stable" includes polycrystalline diamond cutting tables in which abrasive particles (e.g., diamond crystals, etc.) are secured to each other with carbonate binders, as well as cutting tables that consist essentially of diamond, such as cutting tables from which the cobalt has been removed, with or without a silicon or silicon carbide backfill, or that are formed by chemical vapor deposition (CVD) processes.

30 Some embodiments of such methods include preparation of the surface of a substrate to which a cutting table is to be bound before the cutting table is secured to that surface. In specific embodiments, preparation of the surface of the substrate may include removal of one or more contaminants or materials from the surface that may weaken or otherwise interfere with optimal bonding of the cutting table to the surface. In other specific embodiments, a substrate surface may be prepared to receive a cutting table by increasing a porosity or an area of the surface.

40 In such methods, preformed cutting tables, which are also referred to herein as "wafers," are secured, under HTHP conditions, to substrates (e.g., tungsten carbide, etc.) with an intermediate layer of diamond grit. In some embodiments, a powder, particles, or a thin element (e.g., foil, etc.) comprising cobalt or another suitable binder may be used with the diamond grit. In other embodiments, cobalt or another suitable binder material that is present (e.g., as part of a binder, etc.) in the substrate may be caused to sweep into the cutting table as heat and pressure are applied to the cutting table. In further embodiments, a preformed diamond wafer formed by a CVD process may be disposed on a surface of a conventional PDC cutting table previously formed on a substrate. The CVD wafer may then be bonded to the PDC cutting table under HTHP conditions.

55 The present disclosure also includes various embodiments of cutting elements. One embodiment of a cutting element according to the present disclosure includes a substrate, a thermally stable cutting table and an adhesion layer therebetween. The adhesion layer includes diamond particles bonded to the diamonds of the thermally stable cutting table and to the substrate. In addition to diamond, the adhesion layer may include cobalt. The substrate may comprise a cemented carbide, such as tungsten carbide with a suitable binder, such as cobalt. In another embodiment, a preformed cutting table comprising CVD diamond and bonded to a PDC layer comprising cobalt under HTHP conditions is carried by a cemented carbide substrate.

Other features and aspects, as well as advantages, of embodiments of the present disclosure will become apparent to those of ordinary skill in the art through consideration of the ensuing description, the accompanying drawings, and the appended claims.

#### BRIEF DESCRIPTION OF THE DRAWINGS

In the drawings:

FIGS. 1 and 1A illustrate an embodiment of a process for manufacturing PDC cutting elements from preformed cutting tables, with a specific embodiment of preformed cutting table being shown;

FIG. 1B depicts another specific embodiment of a preformed cutting table that may be used to manufacture a PDC cutting element in accordance with various embodiments of teachings of the present disclosure;

FIG. 2 is a carbon phase diagram;

FIG. 3 depicts a PDC cutting element that includes a substrate, a preformed cutting table, and a diamond adhesion layer between the substrate and the preformed cutting table;

FIGS. 4 and 4A depict another embodiment of a process for manufacturing cutting elements that include preformed wafers that consist of diamond;

FIG. 5 illustrates an embodiment of a cutting element that includes a substrate, a PDC cutting table, and a wafer that consists of diamond atop the PDC cutting table; and

FIG. 6 shows an embodiment of an earth-boring rotary drill bit including at least one PDC cutting element that incorporates teachings of the present disclosure.

#### DETAILED DESCRIPTION

With reference to FIG. 1, an embodiment of a process for securing a preformed cutting table 20 to a substrate 30 is illustrated. In that process, at least one "cutter set," which includes a substrate 30 and its corresponding preformed cutting table 20, is assembled.

In the method of FIGS. 1 and 1A, at least one substrate 30 is introduced into a canister assembly, or synthesis cell assembly 50, formed from a refractory metal or other material that will withstand and substantially maintain its integrity (e.g., shape and dimensions) when subjected to HTHP processing. Each substrate 30 may comprise a cemented carbide (e.g., tungsten carbide) substrate for a PDC cutting element, or any other material that is known to be useful as a substrate for PDC cutting elements. In some embodiments, substrate 30 may include a binder material, such as cobalt.

Particles 40 of diamond grit are placed on substrate 30. More specifically, particles 40 are placed on a surface 32 to which a preformed cutting table 20 is to be secured. Particles 40 may be placed on surface 32 alone or with a fine powder or particles 42 of a suitable, known binder material, such as cobalt, another Group VIII metal, such as nickel or iron, or alloys including these materials (e.g., Ni/Co, Co/Mn, Co/Ti, Co/Ni/V, Co/Ni, Fe/Co, Fe/Mn, Fe/Ni, Fe (Ni.Cr), Fe/Si<sub>2</sub>, Ni/Mn, Ni/Cr, etc.).

Surface 32 may be processed to enhance subsequent adhesion of a preformed cutting table 20 thereto. Such processing of surface 32 may, in some embodiments, include removal of one or more contaminants or materials that may weaken or otherwise interfere with optimal bonding of cutting table 20 to surface 32. In specific embodiments, metal carbonate binder, silicon, and/or silicon carbide may be removed from surface 32 of substrate 30, as these materials may inhibit diamond-to-diamond intergrowth, which is desirable for adhering preformed cutting table 20 to surface 32 of substrate

30. The removal of such materials may be effected substantially at surface 32. In such embodiments, one or more materials may be removed to a depth, from surface 32 into substrate 30, that is about the same as a dimension of a diamond particle of preformed cutting table 20, or to a depth of about one micron to about ten microns. In other embodiments, the removal of undesirable materials may extend beyond surface 32, and into substrate 30. Such preparation, in even more specific embodiments, may include leaching of one or more materials from the surface of the substrate.

In other embodiments, an area of surface 32 of substrate 30 may be increased. Chemical, electrical, and/or mechanical processes may, in some embodiments, be used to increase the area of surface 32 by removing material from surface 32. Specific embodiments of techniques for increasing the area of surface 32 include, but are not limited to, laser ablation of surface 32, blasting surface 32 with abrasive material, and exposing surface 32 to chemically etchants.

The removal of such materials may, in some embodiments, enable cobalt or another binder to penetrate into substrate 30 to facilitate the bonding of preformed cutting table 20 to surface 32.

A base surface 22 of preformed cutting table 20 is placed over particles 40 on surface 32 of substrate 30. Base surface 22 of preformed cutting table 20 is of a complementary topography to the topography of surface 32 of substrate 30. Preformed cutting table 20 may be substantially free of metallic binder.

Without limiting the scope of the present disclosure, preformed cutting table 20, in one embodiment, may comprise a PDC with abrasive particles that are bound together with a carbonate (e.g., calcium carbonate, a metallic carbonate (e.g., magnesium carbonate (MgCO<sub>3</sub>), barium carbonate (BaCO<sub>3</sub>), strontium carbonate (SrCO<sub>3</sub>), etc.) binder, etc.). Despite the extremely high pressure and extremely high temperature that are required to fabricate PDCs that include calcium carbonate binders, as this type of PDC is fabricated without a substrate (i.e., is free-standing), it may be formed with standard cutting table dimensions (e.g., diameter and thickness) in a suitable HPHT apparatus, as known in the art.

In another embodiment, depicted by FIG. 1B, a preformed cutting table 20' may comprise a PDC having a face portion 27' and a base portion 23'. Face portion 27' of preformed cutting table 20' is adjacent to and includes a cutting surface 26', which may be filled with silicon and/or silicon carbide. Base portion 23' of preformed cutting table 20' is adjacent to and includes a base surface 22', which consists essentially of diamond. Such an embodiment of preformed cutting element may be manufactured by removing (e.g., by leaching, electrolytic processes, etc.) cobalt or other binder material (e.g., another Group VIII metal, such as nickel or iron, or alloys including these materials, such as Ni/Co, Co/Mn, Co/Ti, Co/Ni/V, Co/Ni, Fe/Co, Fe/Mn, Fe/Ni, Fe (Ni.Cr), Fe/Si<sub>2</sub>, Ni/Mn, and Ni/Cr) from face portion 27' without leaching binder material from base portion 23'. This may be accomplished, for example, by preventing exposure of base portion 23' to leaching conditions and limiting the duration of the leaching conditions. Silicon or silicon carbide is then introduced into the pores that result from the leaching process, such as by the processes described in U.S. Pat. Nos. 4,151,686 and 4,793,828, the entire disclosures of both of which are hereby incorporated herein by this reference. Thereafter, binder material may be leached from base portion 23', leaving pores therein or the binder material may remain. The porous base surface 22' is placed adjacent the surface 32 of substrate 30 (FIGS. 1 and 1A).

With returned reference to FIGS. 1 and 1A, if desired, one or more other cutter sets 12 including a preformed cutting table 20, a quantity of diamond grit particles 40 (and, optionally, binder material powder or particles 42), and a substrate 30 may then be introduced into synthesis cell assembly 50 so that a plurality of cutting elements may be manufactured with a single HTHP process. In embodiments where multiple cutter sets 12 are introduced into a single synthesis cell assembly 50, the order of components of each cutter set 12 may be reversed from the order of components of each adjacent cutter set 12. The cutter sets 12 that are located at ends 52 and 54 of a synthesis cell assembly 50 may be arranged with substrates 30 at ends 52 and 54, or as the outermost elements, to minimize impact upon and the potential for damage to the expensive preformed cutting tables 20.

Once each cutter set 12 has been assembled within synthesis cell assembly 50, the contents of synthesis cell assembly 50 may be subjected to known HTHP processes. The temperature and pressure of such processes are sufficient to cause particles 40 (and, optionally, any binder material powder or particles 42) to bind each preformed cutting table 20 within synthesis cell assembly 50 to its corresponding substrate 30. In some embodiments, the combination of temperature and pressure that are employed in the HTHP process are within the so-called "diamond stable" phase of carbon. A carbon phase diagram, which illustrates the various phases of carbon, including the diamond stable phase D, and the temperatures and pressures at which such phases occur, is provided as FIG. 2.

An embodiment of a PDC cutting element 10 resulting from such processing is shown in FIG. 3. PDC cutting element 10 includes substrate 30, a binder layer 45, and preformed cutting table 20. Binder layer 45 secures preformed cutting table 20 to substrate 30, and may be bonded to preformed cutting table 20 and integrated into the material of substrate 30 at surface 32 (see FIGS. 1 and 1A). In some embodiments, binder layer 45 consists of diamond (e.g., polycrystalline diamond (PCD)). In other embodiments, binder layer 45 consists essentially of diamond. Other embodiments of binder layer 45 include diamond and lesser amounts of a suitable binder material.

In another embodiment of a method encompassed by the present disclosure, which is shown in FIGS. 4 and 4A, at least one cutting element 110 that includes a substrate 30 with a PDC table 120 already secured thereto is introduced into a synthesis cell assembly 50.

A base surface 142 of preformed wafer 140, which may consist essentially of or consist entirely of diamond that has been deposited by known chemical vapor deposition (CVD) processes, is placed over a surface 122 of PDC table 120. Base surface 142 of preformed wafer 140 is of a complementary topography to the topography of surface 122 of PDC table 120.

As described in reference to the embodiment shown in FIGS. 1 and 1A, one or more other cutter sets 112 including a preformed wafer 140 and a cutting element 110 may be introduced into synthesis cell assembly 50 so that a plurality of cutting elements 110 may be manufactured with a single HTHP process. Once each cutter set 112 has been assembled within synthesis cell assembly 50, the contents of synthesis cell assembly 50 may be subjected to known HTHP processes, as described in reference to FIGS. 1 and 1A.

An embodiment of a cutting element 10' resulting from such processing is shown in FIG. 5. Cutting element 10' includes substrate 30, a PDC table 120, and a performed wafer 140 that consists essentially of, or consists of, diamond. Base surface 142 of preformed wafer 140 may be secured to

surface 122 of PDC table 120 by diamond-to-diamond bonding that occurs during the HTHP process, in which diamond from preformed wafer 140 is bonded with diamond-to-diamond bonding, to diamond crystals of PDC table 120. 5 Although the resulting structure may include cobalt or another binder material that may, if it were present on the face of preformed wafer 140, compromise thermal stability, its presence beneath preformed wafer 140 during use of cutting element 10' is at a location which is not subjected to temperatures that are known to be problematic for cutting tables that include cobalt binders.

Turning now to FIG. 6, an embodiment of a rotary type, earth-boring drill bit 60 of the present disclosure is shown. Among other features that are known in the art, bit 60 includes 15 at least one cutter pocket 62. A cutting element 10, 10' according to an embodiment of the present disclosure is received within cutter pocket 62, with substrate 30 (see FIG. 1) bonded or otherwise secured to the material of bit 60. As used herein, the term "earth-boring drill bit" includes without limitation conventional rotary fixed cutter, or "drag" bits, fixed cutter core bits, eccentric bits, bicenter bits, reamer wings, underreamers, roller cone bits, and hybrid bits including both fixed and movable cutting structures, as well as other earth-boring tools configured with cutting structures according to embodiments of the disclosure.

Although the foregoing description contains many specifics, these should not be construed as limiting the scope of the present disclosure, but merely as providing illustrations of some embodiments. Similarly, other embodiments of the disclosure may be devised which do not exceed the scope of the present disclosure. Features from different embodiments may be employed in combination. The scope of specifically claimed embodiments encompassed by this disclosure is, therefore, indicated and limited only by the appended claims and their legal equivalents, rather than by the foregoing description. All additions, deletions and modifications to the embodiments disclosed herein which fall within the meaning and scope of the claims are to be embraced thereby.

What is claimed is:

1. A cutting element for an earth-boring drill bit, comprising:

a thermally stable cutting table comprising a polycrystalline diamond material, the polycrystalline diamond material consisting essentially of a matrix of diamond particles bonded to one another and a silicon, silicon carbide, or silicon and silicon carbide material located within interstitial spaces among interbonded diamond particles of the matrix of diamond particles, the cutting table being at least substantially free of Group VIII metal or alloy catalyst material;

a substrate; and

an adhesion material between and bonded to the cutting table and the substrate, wherein the adhesion material comprises a polycrystalline diamond material bonded to the cutting table and the substrate, the adhesion material being formed separately from formation of the preformed cutting table.

2. The cutting element of claim 1, wherein the polycrystalline diamond material of the thermally stable cutting table consists essentially of the matrix of diamond particles bonded to one another and a silicon material located within the interstitial spaces among the interbonded diamond particles of the matrix of diamond particles.

3. The cutting element of claim 1, wherein the polycrystalline diamond material of the thermally stable cutting table consists essentially of the matrix of diamond particles bonded to one another and a silicon carbide material located within

the interstitial spaces among the interbonded diamond particles of the matrix of diamond particles.

4. The cutting element of claim 1, wherein the adhesion material comprises a Group VIII metal or alloy catalyst material located within interstitial spaces among diamond particles of the adhesion material. 5

5. The cutting element of claim 4, wherein the Group VIII metal or alloy catalyst material comprises cobalt.

6. The cutting element of claim 1, wherein the substrate comprises a Group-VIII-metal- or -alloy-cemented carbide material. 10

7. The cutting element of claim 6, wherein the Group-VIII-metal- or -alloy-cemented carbide material comprises cobalt-cemented tungsten carbide.

8. An earth-boring drill bit, comprising:

a bit body; and

a cutting element secured to the bit body, the cutting element comprising:

a thermally stable cutting table comprising a polycrystalline diamond material, the polycrystalline diamond material consisting essentially of a matrix of diamond particles bonded to one another and a silicon or silicon carbide material located within interstitial spaces among interbonded diamond particles of the matrix of diamond particles, the cutting table being at least substantially free of Group VIII metal or alloy catalyst material;

a substrate secured to the bit body; and

an adhesion material between and bonded to the cutting table and the substrate, wherein the adhesion material comprises a polycrystalline diamond material bonded to the cutting table and the substrate, the adhesion material being formed separately from formation of the preformed cutting table. 25

9. The earth-boring drill bit of claim 8, wherein the adhesion material comprises a Group VIII metal or alloy catalyst material located within interstitial spaces among diamond particles of the adhesion material.

10. The earth-boring drill bit of claim 9, wherein the Group VIII metal or alloy catalyst material comprises cobalt. 40

11. The cutting element of claim 8, wherein the substrate comprises a Group-VIII-metal- or -alloy-cemented carbide material.

12. The cutting element of claim 11, wherein the Group-VIII-metal- or -alloy-cemented carbide material comprises cobalt-cemented tungsten carbide. 45

13. A method of forming a cutting element for an earth-boring drill bit, comprising:

positioning unsintered diamond particles between a substrate and a thermally stable cutting table, the thermally stable cutting table comprising a polycrystalline dia-

mond material, the polycrystalline diamond material consisting essentially of a matrix of diamond particles bonded to one another and a silicon or silicon carbide material located within interstitial spaces among interbonded diamond particles of the matrix of diamond particles, the cutting table being at least substantially free of Group VIII metal or alloy catalyst material; and

subsequently sintering the diamond particles between the substrate and the cutting table to bond the diamond particles to one another, forming an adhesion material, and to bond the adhesion material to the cutting table and the substrate.

14. The method of claim 13, further comprising removing Group VIII metal or alloy catalyst material from the cutting table and introducing the silicon or silicon carbide material into the interstitial spaces among interbonded diamond particles of the matrix of diamond particles of the cutting table before positioning the diamond particles between the substrate and the cutting table. 15

15. The method of claim 13, further comprising positioning particles of a Group VIII metal or alloy catalyst material with the diamond particles between the substrate and the cutting table.

16. The method of claim 15, wherein positioning particles of a Group VIII metal or alloy catalyst material with the diamond particles between the substrate and the cutting table comprises positioning particles of cobalt with the diamond particles between the substrate and the cutting table. 20

17. The method of claim 13, further comprising removing material from a surface of the substrate which the diamond particles are subsequently positioned adjacent to.

18. The method of claim 13, wherein sintering the diamond particles between the substrate and the cutting table comprises subjecting the diamond particles, the substrate, and the cutting table to high-temperature, high-pressure conditions in which carbon is diamond stable. 25

19. The method of claim 13, wherein sintering the diamond particles between the substrate and the cutting table comprises infiltrating a Group VIII metal or alloy catalyst material from the substrate among the diamond particles between the substrate and the cutting table. 40

20. The method of claim 13, wherein positioning the diamond particles between the substrate and the thermally stable cutting table comprises positioning the diamond particles between the substrate and the thermally stable cutting table, the substrate comprising a Group-VIII-metal- or -alloy-cemented carbide material. 45

\* \* \* \* \*